

Jan. 19, 1926.

1,570,064

A. J. JACKMAN

METHOD OF MAKING CRUCIBLES

Filed March 18, 1925

*Fig. 1.*



*Fig. 2.*



*Fig. 3.*



*Fig. 4.*



INVENTOR

Arthur J. Jackman

by his attorneys

Byrnes, Ettinger & Parneller.

## UNITED STATES PATENT OFFICE.

ARTHUR JOHN JACKMAN, OF FOREST HILLS BOROUGH, PENNSYLVANIA, ASSIGNOR  
TO VESUVIUS CRUCIBLE COMPANY, OF SWISSVALE, PENNSYLVANIA, A CORPORA-  
TION OF PENNSYLVANIA.

## METHOD OF MAKING CRUCIBLES.

Application filed March 18, 1925. Serial No. 16,344.

*To all whom it may concern:*

Be it known that I, ARTHUR JOHN JACKMAN, a citizen of the United States, residing at Forest Hills Borough, county of Allegheny, and State of Pennsylvania, have invented a new and useful Improvement in Methods of Making Crucibles, of which the following is a full, clear, and exact description.

10 The present invention pertains to a method of making crucibles and is particularly adapted to the manufacture of graphite crucibles such as are used in the manufacture of steel.

15 Metal melting crucibles, as for example, graphite crucibles used in steel manufacture, are subjected to internal erosion of three principal sorts; namely, the oxidation of the graphite by available oxygen in the bath, the absorption of carbon from the crucible by the metal, and the fluxing action of the slag on the material used to bond the crucible. This last constitutes a very destructive localized attack.

25 Heretofore it has been common practice to line such crucibles with various materials, possessing greater resistance than the body of the crucible to the corrosive action of the slag, to obtain greater life for the crucibles

30 or to obtain carbon free metal. Complete linings have been found unsatisfactory, however, because of the irregularity of the amount of carbon absorbed by the metal when the lining becomes cracked, a circumstance which eventually obtains.

35 The repair of eroded crucibles has also been tried. The repairs have been made by filling the crack or groove formed in the crucible with a material similar to that of which the crucible or crucible lining is made. This procedure has not always proved effective because the first heat of service renders a crucible hard burned and vitreous, and material subsequently filled 40 into cracks or grooves in the surface of such a crucible cannot become firmly bonded thereto. In addition to this, the usual practice in crucible steel furnace operation is to charge the crucibles while yet hot from the 45 previous heat and put them back into the furnace. Under such operating conditions patching is impracticable.

50 Avoiding these objections and producing a crucible of longer life than those hitherto

manufactured, my invention provides for 55 incorporating a protecting ring of slag resisting material in the interior of the crucible at the time it is manufactured. Thus I am able to produce a crucible presenting a monolithic body of graphitic composition 60 to the bulk of the metal, at the same time presenting to the slag a protective ring of a composition best suited to resist the fluxing action of the same.

65 In making these protective rings I preferably employ such materials as chromite, sillimanite, zirconia, spinel, zircon, or compositions containing one or more of these ingredients. It will be understood, however, that I am not limited to these materials, 70 since it is obvious that any highly refractory substance that is neutral and resistant to the fluxing action of the slags encountered will serve my purpose. I may also employ graphite in these rings in order that 75 the thermal and physical proportions of the rings will more closely approximate those of the crucible body. These protecting rings may be bonded with any suitable bonding material, such as those now well known in 80 the art.

85 In the accompanying drawings, illustrating the present preferred embodiment of the invention—

Figure 1 is a vertical section of a crucible having a ring cut in the inner surface in the vicinity of the slag line;

Figure 2 is a cross sectional view of a crucible provided with a retaining groove having the side portions undercut;

Figure 3 is a sectional view to enlarged scale, illustrating a portion of the crucible shown in Figure 2 with the protecting material in place;

Figure 4 illustrates a slag resisting ring 95 similar to that shown in Figure 3 but provided with a protective coating to prevent abrasion of the inlay until the crucible is hard burned.

Referring first to Figure 1, there is shown 100 a crucible 2 having an annular groove 3 whose side walls 4 are cut substantially perpendicular to the inner surface of the crucible wall. The groove 3 is preferably cut while the crucible is soft and unburned. I 105 have found that the depth of this groove 3 should not be greater than two-thirds the thickness of the crucible wall. Greater

depth of cut adds no mechanical strength to the finished slag resisting ring and may seriously weaken the crucible.

Figure 2 illustrates a crucible 2<sup>a</sup> having 5 a retaining groove 5 cut therein. This groove 5 has sloping sides 6 which effectively retain the material 7 packed in the groove, as better shown in Figure 3. In practice it is found that the width of such a groove 10 need not exceed eight inches, as the depth of the slags encountered does not warrant it. It will be understood, however, that this dimension is not to be construed as a limit.

In constructing such a crucible as shown 15 in Figure 3 it is desirable that the slag resisting material 7 should have contact with the side walls 6 and the inner wall 8 to insure the material 7 being firmly held in place. It is obvious that if the material 7 has a 20 smaller shrinkage than the crucible wall 2' it will be crushed during drying or firing. To obviate this difficulty, I prefer to form the crucible body and permit it to partially dry before the slag ring is molded into the 25 groove. When this is done the differential in shrinkage between the crucible body 2' and the slag resisting material 7 is reduced to practically nothing.

Certain of the desirable slag resisting materials, such as water ground zirconia without added bonding material, do not possess much physical strength or resistance to abrasion until they have been sintered at higher temperatures than those usually employed in the manufacture of graphite crucibles. When it is necessary to depend upon the heat of the steel furnace to give such materials a final firing, I provide for coating the exposed portion of the ring with a 30 ceramic composition to protect it from abrasion. In Figure 4 such a composition 9 is shown extending above and below the slag resisting material 7, making contact with the crucible body 2'. For such a composition 9, I preferably employ a mix sufficiently 35 similar to that used in the crucible body 2' that a good bond is secured therewith above and below the slag ring, thus insuring protection of the slag ring until the crucible 40 has been hard burned. The protective coating 9 is soon destroyed during the early use of the crucible and the slag resisting ring 45 performs its function as above described.

While I have described the preferred embodiment of the invention, it will be understood that the drawings do not define the limits of the invention, which may be otherwise embodied within the scope of the following claims.

60 I claim:

1. As an article of manufacture, a crucible for a melting operation wherein a slag is formed, having a portion adapted to contact with the slag and made from a material 65 more resistant than the body of the crucible

to the corrosive action of the slag, substantially as described.

2. As an article of manufacture, a crucible for a metal melting operation wherein slag is formed, having a graphitic body portion adapted to contact with the bulk of the metal and having a portion adapted to contact with the slag and made from a material more resistant than the said body portion to the corrosive action of the slag, substantially 70 as described. 75

3. As an article of manufacture, a crucible for an operation wherein slag is formed, having an inlay of refractory material more resistant than the body of the crucible to 80 the corrosive action of the slag, substantially as described.

4. As an article of manufacture, a crucible for an operation wherein slag is formed, comprising a body portion of refractory material and having an interior ring of material more resistant to the chemical attack of the slag than the said body portion incorporated therein at such portions as normally contact with the slag, substantially 90 as described. 95

5. As an article of manufacture, a crucible for an operation wherein slag is formed, comprising a body portion of graphitic material and having an interior ring of material more resistant to the chemical attack of the slag than the said body portion incorporated therein at such portions as normally contact with the slag, substantially as 100 described. 105

6. As an article of manufacture, a crucible for an operation wherein slag is formed, comprising a graphite body, means for protecting the said body portion from the corrosive action of the slag comprising an inlay of material more resistant to the chemical attack of the slag than the body portion, and means for protecting the inlaid material from injury prior to hard burning, comprising a veneer of refractory material placed thereover, substantially as described. 110

7. As an article of manufacture, a crucible for an operation wherein slag is formed, comprising a graphite body, means for protecting the said body portion from the corrosive action of the slag comprising an inlay of material more resistant to the chemical attack of the slag than the body portion, and means for protecting the inlaid material from injury prior to hard burning, comprising a veneer of refractory material overburned at a relatively lower temperature than required for hard burning the inlaid material, substantially as described. 115 120

8. As an article of manufacture, a crucible for an operation wherein slag is formed, having a graphitic body portion, means for protecting the body portion from the corrosive action of the slag comprising an annular ring of refractory material, more re- 125 130

sistant to the attack of the slag than the body portion, inlaid in the body portion at such portions thereof as are normally in contact with the slag, and means for protecting the said inlaid material from injury prior to hard burning comprising a thin layer of material placed over the said inlaid material and bonded to the said body portion, substantially as described.

10 9. The method of making a crucible for an operation wherein slag is formed comprising forming a body portion having a groove therein at the slag zone, and thereafter packing the groove with material more 15 resistant than the body portion to the corrosive action of the slag, substantially as described.

10 10. The method of making a crucible for an operation wherein slag is formed comprising forming a body portion having an annular groove, whose width is greater at the bottom thereof than at the top, at the region normally in contact with the slag, thereafter packing said groove with material more 25 resistant to the chemical attack of the slag than the body portion, and placing thereover a layer of material adapted to protect the inlaid material from injury prior to hard burning, substantially as described.

30 11. The method of making a graphite crucible for an operation wherein slag is formed comprising forming a body portion having an annular groove, whose width is greater at the bottom thereof than at the 35 top, at the region normally in contact with the slag, thereafter packing said groove with material more resistant to the chemical attack of the slag than the body portion, placing thereover a layer of material adapted 40 to protect the inlaid material from injury prior to hard burning, and firing the crucible so made, substantially as described.

12. The method of incorporating a slag resisting portion having a relatively low 45 drying shrinkage into a crucible having a relatively higher drying shrinkage comprising

ing forming the crucible to a desired shape and drying the same until a predetermined proportion of the total shrinkage has taken place, and thereafter introducing the slag 50 resisting portion into the said crucible, substantially as described.

13. The method of incorporating a slag resisting portion having a relatively low drying shrinkage into a crucible having a 55 relatively higher drying shrinkage comprising forming the crucible to a desired shape and drying the same until a predetermined proportion of the total shrinkage has taken place, thereafter introducing the slag resisting portion into the said crucible, and placing thereover a material adapted to protect the slag resisting portion from injury prior to hard burning, substantially as described.

14. The method of incorporating a slag resisting ring having a relatively low drying shrinkage into a graphite crucible having a relatively higher drying shrinkage comprising forming the graphite crucible to a desired shape and drying the same until a 70 predetermined proportion of the total shrinkage has taken place, and thereafter introducing the slag resisting ring into the said graphite crucible, substantially as described.

15. The method of incorporating a slag resisting ring having a relatively low drying shrinkage into a graphite crucible having a relatively higher drying shrinkage comprising forming the crucible to a desired shape and drying the same until a predetermined proportion of the total shrinkage has taken place, thereafter introducing the slag resisting ring into the said crucible, and placing thereover a material adapted to protect the slag resisting ring from injury prior to hard burning, substantially as described.

In testimony whereof I have hereunto set my hand.

ARTHUR JOHN JACKMAN.